# EUROPEAN PATENT SPECIFICATION

(11) **EP 2 664 416 B1**
(45) Date of publication and mention of the grant of the patent: **02.09.2015**
(21) Application number: 13168211.4
(22) Date of filing: 17.05.2013
(51) Int. Cl.: B24D 18/00

(54) **Method of manufacturing an abrasive tool**
Verfahren zur Herstellung eines Schleifwerkzeugs
Procédé de fabrication d'un outil abrasif

(30) Priority: 17.05.2012 IT VR20120097
(43) Date of publication of application: 20.11.2013
(73) Proprietor: Mirani, Willem, 37010 Cavaion Veronese (VR) (IT)
(72) Inventor: Mirani, Willem, 37010 Cavaion Veronese (VR) (IT)
(74) Representative: Modiano, Micaela Nadia

(56) References cited:
- FR-A- 1 179 314

## Description

The present invention relates to a method for manufacturing an abrasive tool.

Typically, abrasive tools are constituted by a metallic supporting body, which is for example disk-shaped and has a working surface that supports the abrasive powder.

The supporting body is mounted on a machine tool, for example a sanding machine, which transmits to the tool a motion, typically a cyclic, linear, oscillating or rotary motion, so as to move the working surface into contact with the part to be machined.

The tool can also be stationary, such as for example a lathe tool.

Known abrasive tools, for example backing pads, are constituted by a metallic supporting body, typically made of steel, that has a working surface covered by a layer of abrasive powders (for example diamond powder) mixed with a bonding substance, such as for example an adhesive.

Although these constructive solutions are used extensively, they are not free from drawbacks.

First of all, the use of bonding agents leads to a lower efficiency of the abrasive capacity of the working surface.

Secondly, in order to ensure a stable grip of the abrasive powder and of the bonding agent to the working surface, supporting bodies made of steel of considerable weight are often used: this causes an increase in the operating costs of the abrasive tool as well as vibrations.

FR 1 179 314 A discloses a method for manufacturing an abrasive tool including the steps as defined in the pre-characterising postion of the appended claim 1.

The aim of the present invention is to eliminate or at least reduce drastically the drawbacks described above.

Within this aim, an object of the invention is to provide a method for manufacturing an abrasive tool that makes it possible to obtain an abrasive tool without using bonding agents or adhesives.

A further object of the invention is to provide a method for manufacturing an abrasive tool that is extremely lightweight, so as to reduce the operating costs and the risk of the onset of vibrations.

This aim, as well as these and other objects that will become more apparent hereinafter, are achieved by a method for manufacturing an abrasive tool according to claim 1.

Further characteristics and advantages of the invention will become more apparent from the description of some preferred but not exclusive embodiments of a method for manufacturing an abrasive tool according to the invention, illustrated by way of non-limiting example in the accompanying drawings, wherein:
Figure 1 is a sectional view of an abrasive tool obtained by means of the method according to the invention.

The present invention relates to a method for manufacturing an abrasive tool, generally designated by the reference numeral 1. The method comprises:
- a step of depositing, on a working surface 2a formed on a metallic supporting body 2, an abrasive powder 3;
- a step of heating the working surface 2a and the abrasive powder 3 to a temperature above 400 °C;
- a step of pressing the abrasive powder 3 against the working surface 2a at a pressure of more than 0.75 t/cm²;
- a step of cooling the metallic supporting body 2 in oil in a time comprised between 2.5 minutes and 10 minutes.

Advantageously, the abrasive powder 3 is selected from the group that comprises:
- diamond powder;
- synthetic diamond powder;
- super-abrasive powder;
- molten carbides of tungsten, titanium, tantalum (widia);
- zirconium;
or mixtures thereof.

Conveniently, the metallic supporting body 2 is made of aluminum or alloys thereof.

It has been found that it is particularly advantageous for the heating step to comprise heating to a temperature above 520 °C and preferably comprised between 545 °C and 555 °C.

The step of pressing the abrasive powder against the working surface is performed preferably at a pressure of more than 1.45 t/cm² and preferably substantially equal to 1.50 t/cm².

By way of example, the heating step can be performed at a temperature comprised between 400 °C and 600 °C while the pressing step provides for a pressure comprised between 0.75 t/cm² and 2 t/cm².

In this regard it has been observed experimentally that by increasing the temperature at which the heating step is performed it is possible to use pressures that correspond to the lowest values of the range cited above, whereas by decreasing the temperature at which the heating step is performed it is necessary to use pressures that correspond to the highest values of the range cited above.

Advantageously, the step of cooling the metallic supporting body 2 in oil is performed in a time comprised between 4 minutes and 6 minutes and preferably over a time substantially equal to 5 minutes.

As shown, the method according to the invention has been found to be extremely satisfactory for the production of abrasive tools 1 of any shape and type, such as, merely by way of example, backing pads, cutters (cylindrical, spherical, conical, etc.), files, floats, including fixed ones, etcetera.

According to a further aspect, the present invention relates to an abrasive tool 1 that is provided by means of a method according to what has been described above.

All the characteristics of the invention indicated above as advantageous, convenient or the like may also be omitted or be replaced with equivalents.

The individual characteristics presented with reference to general teachings or to particular embodiments may all be present in other embodiments or may replace characteristics in these embodiments.

In practice it has been found that the invention has achieved the intended aim and objects in all of its embodiments.

In particular, it has been found that an abrasive tool 1 obtained by means of the method according to the invention has a significantly longer life than currently commercially available tools.

Moreover, by using the process parameters cited above it has been found surprisingly that it is possible to fix the abrasive powder to a metallic body made of aluminum or aluminum alloy, thus reducing the vibrations and overheating of the abrasive tool during its use.

All the details may further be replaced with other technically equivalent elements.

In practice, the materials used, as well as the contingent shapes and dimensions, may be any according to requirements and to the state of the art.

Where technical features mentioned in any claim are followed by reference signs, those reference signs have been included for the sole purpose of increasing the intelligibility of the claims and accordingly such reference signs do not have any limiting effect on the interpretation of each element identified by way of example by such reference signs.

## Claims

1. A method for manufacturing an abrasive tool (1), comprising the steps that consist in:
- depositing, on a working surface (2a) formed on a metallic supporting body (2), an abrasive powder (3) without using binders or adhesives;
- heating said working surface (2a) and said abrasive powder (3) to a temperature above 400 °C;
- pressing said abrasive powder (3) against said working surface (2a);
- cooling said metallic supporting body (2);
the method being **characterized in that** the step of pressing said abrasive powder (3) against said working surface (2a) is performed with a pressure of more than 0.75 t/cm², and **in that** the step of cooling said metallic supporting body (2) is performed in oil in a time comprised between 2.5 minutes and 10 minutes.

2. The method according to claim 1, **characterized in that** said abrasive powder (3) is selected from the group that comprises:
- diamond powder;
- synthetic diamond powder;
- super-abrasive powder;
- molten carbides of tungsten, titanium, tantalum (widia);
- zirconium;
or mixtures thereof.

3. The method according to one of the preceding claims, **characterized in that** said metallic supporting body (2) is made of aluminum or alloys thereof.

4. The method according to one of the preceding claims, **characterized in that** said heating step comprises heating to a temperature above 520 °C and preferably comprised between 545 °C and 555 °C.

5. The method according to one of the preceding claims, **characterized in that** said step of pressing said abrasive powder (3) against said working surface (2a) is performed at a pressure of more than 1.25 t/cm² and preferably substantially equal to 1.50 t/cm².

6. The method according to one of the preceding claims, **characterized in that** said step of cooling said metallic supporting body (2) in oil is performed in a time comprised between 4 minutes and 6 minutes and preferably in a time substantially equal to 5 minutes.

7. The method according to one of the preceding claims, **characterized in that** said abrasive tool (1) is selected from the group that comprises:
- a backing pad;
- a cutter (cylindrical, spherical, conical, etcetera);
- a file;
- a float;
or the like.

## Patentansprüche

1. Ein Verfahren zur Herstellung eines Schleifwerkzeugs (1), das folgende Schritte umfasst:
- Auftragen eines Schleifpulvers (3), ohne Verwendung von Bindemitteln oder Klebstoffen, auf eine Arbeitsoberfläche (2a), die auf einem metallischen Trägerkörper (2) geformt ist;
- Erhitzen der Arbeitsoberfläche (2a) und des Schleifpulvers (3) auf eine Temperatur oberhalb von 400°C;
- Drücken des Schleifpulvers (3) gegen die Arbeitsoberfläche (2a);
- Kühlen des metallischen Trägerkörpers (2);
wobei das Verfahren **dadurch gekennzeichnet ist, dass** der Schritt des Drückens des Schleifpulvers (3) gegen die Arbeitsoberfläche (2a) mit einem Druck von mehr als 0,75 t/cm² durchgeführt wird, und dadurch, dass der Schritt des Kühlens des metallischen Trägerkörpers (2) in Öl in einer Zeit zwischen 2,5 Minuten und 10 Minuten durchgeführt wird.

2. Das Verfahren gemäß Anspruch 1, **dadurch gekennzeichnet, dass** das Schleifpulver (3) gewählt ist aus der Gruppe, die Folgendes umfasst:
- Diamantpulver,
- synthetisches Diamantpulver,
- Super-Abrasions-Pulver,
- geschmolzene Carbide von Wolfram, Titan, Tantal (Widia),
- Zirkonium
oder Mischungen davon.

3. Das Verfahren gemäß einem der obigen Ansprüche, **dadurch gekennzeichnet, dass** der metallische Trägerkörper (2) aus Aluminium oder Legierungen davon besteht.

4. Das Verfahren gemäß einem der obigen Ansprüche, **dadurch gekennzeichnet, dass** der Erhitzungsschritt das Erhitzen auf eine Temperatur oberhalb von 520°C und vorzugsweise zwischen 545°C und 555°C umfasst.

5. Das Verfahren gemäß einem der obigen Ansprüche, **dadurch gekennzeichnet, dass** der Schritt des Drückens des Schleifpulvers (3) gegen die Arbeitsoberfläche (2a) mit einem Druck von mehr als 1,25 t/cm² und vorzugsweise im Wesentlichen gleich 1,50 t/cm² durchgeführt wird.

6. Das Verfahren gemäß einem der obigen Ansprüche **dadurch gekennzeichnet, dass** der Schritt des Kühlens des metallischen Trägerkörpers (2) in Öl in einer Zeit zwischen 4 Minuten und 6 Minuten und vorzugsweise in einer Zeit im Wesentlichen gleich 5 Minuten durchgeführt wird.

7. Das Verfahren gemäß einem der obigen Ansprüche, **dadurch gekennzeichnet, dass** das Schleifwerkzeug (1) gewählt ist aus der Gruppe, die Folgendes umfasst:
- eine Träger-Unterlage,
- eine Trennvorrichtung (zylindrisch, kugelförmig, kegelförmig und so weiter),
- eine Feile,
- ein Reibebrett,
oder dergleichen.

## Revendications

1. Procédé de fabrication d'un outil abrasif (1), qui comprend les étapes qui consistent à :
- déposer, sur une surface de travail (2a) formée sur un corps de support métallique (2), une poudre abrasive (3) sans utiliser des liants ou des adhésifs ;
- chauffer ladite surface de travail (2a) et ladite poudre abrasive (3) à une température supérieure à 400°C ;
- presser ladite poudre abrasive (3) contre ladite surface de travail (2a) ;
- refroidir ledit corps de support métallique (2) ;
le procédé étant **caractérisé en ce que** l'étape de pression de ladite poudre abrasive (3) contre ladite surface de travail (2a) est effectuée avec une pression supérieure à 0,75 t/cm², et **en ce que** l'étape de refroidissement dudit corps de support métallique (2) est effectuée dans de l'huile pendant une durée comprise entre 2,5 minutes et 10 minutes.

2. Procédé selon la revendication 1, **caractérisé en ce que** ladite poudre abrasive (3) est choisie parmi le groupe qui comprend :
- de la poudre de diamant ;
- de la poudre de diamant synthétique :
- de la poudre super-abrasive ;
- des carbures fondus de tungstène, de titane, de tantale (widia) ;
- du zirconium ;
ou des mélanges de ceux-ci.

3. Procédé selon l'une des revendications précédentes, **caractérisé en ce que** ledit corps de support métallique (2) est composé d'aluminium ou d'alliages de celui-ci.

4. Procédé selon l'une des revendications précédentes, **caractérisé en ce que** ladite étape de chauffage comprend le chauffage à une température supérieure à 520°C, et de préférence comprise entre 545°C et 555°C.

5. Procédé selon l'une des revendications précédentes, **caractérisé en ce que** ladite étape de pression de ladite poudre abrasive (3) contre ladite surface de travail (2a) est effectuée à une pression supérieure à 1,25 t/cm², et de préférence sensiblement égale à 1,50 t/cm².

6. Procédé selon l'une des revendications précédentes, **caractérisé en ce que** ladite étape de refroidissement dudit corps de support métallique (2) dans de l'huile est effectuée pendant une durée comprise entre 4 minutes et 6 minutes, et de préférence pendant une durée sensiblement égale à 5 minutes.

7. Procédé selon l'une des revendications précédentes, **caractérisé en ce que** ledit outil abrasif (1) est choisi parmi le groupe qui comprend :
- un plateau de ponçage ;
- un cutter (cylindrique, sphérique, conique, etc.) ;
- une lime ;
- une lisseuse ;
ou similaires.
